

1

3,340,051

### TITANIUM-BASE ALLOYS

Evan William Evans, Hagley, and Michael Duncan Smith, Shenstone, England, assignors to Imperial Metal Industries (Kynoch) Limited, London, England, a corporation of Great Britain

No Drawing. Filed Sept. 28, 1964, Ser. No. 399,666  
Claims priority, application Great Britain, Oct. 2, 1963,  
38,828/63

6 Claims. (Cl. 75—175.5)

This invention relates to titanium-base alloys having a high Young's modulus and to a method of heat-treatment for such alloys.

In order to be competitive with steels on the grounds of weight and stiffness, titanium-base alloys require a Young's modulus greater than  $20 \times 10^6$  lbs./sq. in. One alloy which meets this requirement has the nominal composition Ti5-Al1.5-B, but is difficult to process and cracking frequently occurs during hot working. The especial care needed during processing to avoid cracking and the close inspection of the processed alloy required to detect cracked material adds to the cost of production.

The present invention is directed to modified compositions which have greater resistance to cracking during hot working whilst retaining good Young's modulus values and adequate ductility.

According to the invention, a titanium-base alloy consists of up to 10% by weight of chromium and 0.5-2% of boron, balance, apart from usual impurities, titanium.

Also according to the invention, a titanium-base alloy consists of up to 10% by weight of chromium, 3-7% of aluminium, 0.5-2% of boron, balance, apart from usual impurities, titanium, but preferably the alloy contains 4-7% aluminium.

The usual impurity elements include carbon, nitrogen and oxygen, which may be present at the normal commercial levels.

The preferred range of composition for the element chromium is 2-10%.

Alloys in accordance with the invention possess a good combination of high Young's modulus, ultimate tensile strength and ductility, and are easier to process than the Ti5-Al1.5-B alloy since the ductility in hot working is improved. Forgeability is improved, forged stock being free from surface and internal cracks. In the heat-treated condition the alloy is useful in rod and sheet form for structural applications.

Increasing the chromium content increases the modulus but reduces the ductility somewhat and a chromium content of about 5% with a boron content of about 1.2% has been found to give a good combination of Young's modulus and ductility. A further improvement in tensile strength and modulus is obtained when aluminium is added, there being what appears to be a synergistic effect. The chromium content is therefore reduced from that

10

mentioned above when aluminium is present and a Young's modulus of  $21 \times 10^6$  lbs./sq. in. is obtained with 3% chromium, 6% aluminium and 1% boron. Chromium contents as high as 7% produce a further increase in modulus, but ductility is adversely affected. Increasing 15 aluminium and boron content also increases the modulus.

Quaternary alloys tend to give higher values of Young's modulus than ternary alloys, although in both types of alloy, modulus, tensile strength and ductility may be controlled by varying heat-treatment conditions.

In order to develop this desirable combination of properties, the alloys are subjected to a heat-treatment comprising solution-treating at a temperature in the alpha plus beta or the beta field, quenching, and ageing at as high a temperature as possible below the eutectoid temperature.

Solution-treatment may be carried out at about 750° C. in the alpha plus beta field and ageing may be carried out at about 650° C. The period of ageing is important to produce maximum modulus values which, in general, occur in the period 20 to 160 hours, dependent on composition.

Composition affects the duration of ageing treatment and alloys having greater chromium contents age to high modulus more rapidly than the lower chromium contents.

The effects of composition and of various ageing times 25 on Young's modulus are shown in Table I and on the tensile properties in Table II. It will be seen from these tables that certain alloys require a long ageing treatment and others need a shorter treatment, in order to develop a good combination of strength and ductility. The improvement in modulus brought about by the addition of aluminium is clearly demonstrated in Table I.

In general, the ageing of the alloys initially produced an increase in modulus, though rate varied with the composition, and after a maximum modulus was reached, the alloys slowly over-aged. Alloys with high chromium and aluminium content had a considerably higher rate of ageing, maximum modulus being approached after about 18 hours ageing.

The results of tensile tests are shown in Table II. Tensile strength of the alloys of the Ti-Cr-B type is high in the water-quenched condition and falls on ageing. Increase of chromium and boron content increases strength. Prolonged ageing reduces the ductility of these alloys.

Structures of the alloys depend upon the degree of beta stabilisation. The ternary and quaternary alloys with low chromium contents have in the quenched condition equiaxed alpha-beta structures containing boride particles, and structure is not appreciably changed by ageing. Ternary alloys of high chromium content, as quenched, have a structure of boride particles dispersed in a retained beta matrix whilst in the quaternary containing aluminium, the matrix consists of martensitically transformed beta. On ageing, retained beta and martensite alike break down to give fine duplex structures.

30

35

40

45

50

2

mentioned above when aluminium is present and a Young's modulus of  $21 \times 10^6$  lbs./sq. in. is obtained with 3% chromium, 6% aluminium and 1% boron. Chromium contents as high as 7% produce a further increase in modulus, but ductility is adversely affected. Increasing aluminium and boron content also increases the modulus.

Quaternary alloys tend to give higher values of Young's modulus than ternary alloys, although in both types of alloy, modulus, tensile strength and ductility may be controlled by varying heat-treatment conditions.

In order to develop this desirable combination of properties, the alloys are subjected to a heat-treatment comprising solution-treating at a temperature in the alpha plus beta or the beta field, quenching, and ageing at as high a temperature as possible below the eutectoid temperature.

Solution-treatment may be carried out at about 750° C. in the alpha plus beta field and ageing may be carried out at about 650° C. The period of ageing is important to produce maximum modulus values which, in general, occur in the period 20 to 160 hours, dependent on composition.

Composition affects the duration of ageing treatment and alloys having greater chromium contents age to high modulus more rapidly than the lower chromium contents.

The effects of composition and of various ageing times 25 on Young's modulus are shown in Table I and on the tensile properties in Table II. It will be seen from these tables that certain alloys require a long ageing treatment and others need a shorter treatment, in order to develop a good combination of strength and ductility. The improvement in modulus brought about by the addition of aluminium is clearly demonstrated in Table I.

In general, the ageing of the alloys initially produced an increase in modulus, though rate varied with the composition, and after a maximum modulus was reached, the alloys slowly over-aged. Alloys with high chromium and aluminium content had a considerably higher rate of ageing, maximum modulus being approached after about 18 hours ageing.

The results of tensile tests are shown in Table II. Tensile strength of the alloys of the Ti-Cr-B type is high in the water-quenched condition and falls on ageing. Increase of chromium and boron content increases strength. Prolonged ageing reduces the ductility of these alloys.

Structures of the alloys depend upon the degree of beta stabilisation. The ternary and quaternary alloys with low chromium contents have in the quenched condition equiaxed alpha-beta structures containing boride particles, and structure is not appreciably changed by ageing. Ternary alloys of high chromium content, as quenched, have a structure of boride particles dispersed in a retained beta matrix whilst in the quaternary containing aluminium, the matrix consists of martensitically transformed beta. On ageing, retained beta and martensite alike break down to give fine duplex structures.

55

TABLE I.—COMPOSITION AND ELASTIC MODULI OF TITANIUM-CHROMIUM-ALUMINIUM-BORON ALLOYS

| Nominal composition, Wt. percent |    |     | Analysed composition, Wt. percent |      |      | Modulus of elasticity (lbs./sq. in. $\times 10^6$ ) WQ from 750° C. and aged at 65° C. for:—(in hours) |       |       |       |       |       |       |       |       |       |
|----------------------------------|----|-----|-----------------------------------|------|------|--------------------------------------------------------------------------------------------------------|-------|-------|-------|-------|-------|-------|-------|-------|-------|
| Cr                               | Al | B   | Cr                                | Al   | B    | 0                                                                                                      | 1     | 4     | 10    | 17    | 18    | 61½   | 105½  | 155   | 1,188 |
| 5                                | —  | 0.8 | 4.0                               | —    | 0.67 | 18.65                                                                                                  | —     | —     | —     | 17.41 | —     | 18.87 | 18.90 | 18.80 | 17.81 |
| 5                                | —  | 1   | 3.7                               | —    | .81  | 18.53                                                                                                  | —     | —     | —     | 17.31 | —     | 18.68 | 18.76 | 18.65 | 18.23 |
| 5                                | —  | 1.2 | 4.15                              | —    | 1.08 | 19.14                                                                                                  | —     | —     | —     | 18.06 | —     | 19.86 | 19.94 | 19.91 | 17.97 |
| 7                                | —  | 1   | —                                 | —    | —    | 15.71                                                                                                  | 16.59 | 16.64 | 17.46 | —     | 17.79 | —     | —     | —     | —     |
| 9                                | —  | 1   | 5.44                              | —    | 1.03 | 14.58                                                                                                  | 17.62 | 17.01 | 19.06 | —     | 19.31 | —     | —     | —     | —     |
| 3                                | 6  | 0.8 | 2.55                              | 5.59 | 0.75 | 17.66                                                                                                  | —     | —     | —     | 19.52 | —     | 19.75 | 19.83 | 19.84 | 20.61 |
| 3                                | 6  | 1   | 2.6                               | 5.61 | 0.87 | 18.63                                                                                                  | —     | —     | —     | 20.44 | —     | 20.69 | 20.72 | 20.78 | 19.58 |
| 3                                | 6  | 1.2 | 2.55                              | 5.58 | 1.07 | 19.13                                                                                                  | —     | —     | —     | 20.8  | —     | 21.04 | 21.07 | 21.16 | 20.82 |
| 7                                | 6  | 1   | 6.46                              | 5.89 | 0.99 | 17.19                                                                                                  | 20.67 | 21.43 | 21.55 | —     | 21.57 | —     | —     | —     | —     |

TABLE II.—TENSILE PROPERTIES OF TITANIUM-CHROMIUM-ALUMINUM-BORON ALLOYS, WATER-QUENCHED FROM 750° C. AND AGED AT 60° C.

| Nominal Composition, Wt. percent |       |     | Ageing Time, Hours | Hardness, D.P.N. | Tensormeter Yield Stress, t.s.i. | Tensile Strength, t.s.i. | Percent Elong. on 4/A |
|----------------------------------|-------|-----|--------------------|------------------|----------------------------------|--------------------------|-----------------------|
| Cr                               | Al    | B   |                    |                  |                                  |                          |                       |
| 5.0                              | ----- | 0.8 | As WQ              | -----            | 80.4                             | 86.4                     | 5                     |
|                                  |       |     | 61½                | -----            | 44.7                             | 54.4                     | 13                    |
|                                  |       |     | 156                | -----            | 48.8                             | 56.3                     | 19                    |
| 5.0                              | ----- | 1.0 | As WQ              | 422              | 72.0                             | 174.5                    | 2                     |
|                                  |       |     | 61½                | -----            | 79.4                             | 83.9                     | 5                     |
|                                  |       |     | 156                | -----            | 45.7                             | 59.7                     | 14                    |
| 5.0                              | ----- | 1.2 | As WQ              | 358              | 48.8                             | 56.3                     | 20                    |
|                                  |       |     | 61½                | -----            | 62.3                             | 67.4                     | 9                     |
|                                  |       |     | 156                | -----            | (1)                              | 66.8                     | (1)                   |
| 7.0                              | ----- | 1.0 | As WQ              | 441              | 55.7                             | 61.2                     | 8                     |
|                                  |       |     | 61½                | -----            | 57.7                             | 64.8                     | 12                    |
|                                  |       |     | 156                | -----            | 67.4                             | 79.4                     | 6                     |
| 9.0                              | ----- | 1.0 | As WQ              | 393              | 65.4                             | 70.4                     | 12                    |
|                                  |       |     | 20                 | 373              | 62.4                             | 67.9                     | 8                     |
|                                  |       |     | 4                  | 436              | 71.9                             | 79.4                     | 8                     |
| 3.0                              | 6.0   | 0.8 | As WQ              | 373              | 66.3                             | 73.4                     | 7                     |
|                                  |       |     | 20                 | 375              | 61.9                             | 70.9                     | 7                     |
|                                  |       |     | 61½                | -----            | 70.4                             | 76.4                     | 10                    |
| 3.0                              | 6.0   | 1.0 | As WQ              | 391              | 72.5                             | 77.9                     | 3                     |
|                                  |       |     | 61½                | -----            | 73.4                             | 77.9                     | 3                     |
|                                  |       |     | 1,188              | -----            | 71.5                             | 75.0                     | 4                     |
| 3.0                              | 6.0   | 1.2 | As WQ              | 340              | 71.8                             | 78.3                     | 8                     |
|                                  |       |     | 61½                | -----            | 74.7                             | 81.6                     | 6                     |
|                                  |       |     | 156                | -----            | 76.4                             | 81.4                     | 5                     |
| 3.0                              | 6.0   | 1.2 | As WQ              | 414              | 49.5                             | 56.7                     | 18                    |
|                                  |       |     | 61½                | -----            | 76.9                             | 81.9                     | 8                     |
|                                  |       |     | 156                | -----            | (1)                              | 122.9                    | (1)                   |
| 7.0                              | 6.0   | 1.0 | As WQ              | 496              | 74.5                             | 79.7                     | 4                     |
|                                  |       |     | 4                  | 508              | (1)                              | 90.5                     | 5                     |
|                                  |       |     | 20                 | 537              | (1)                              | 76.9                     | (1)                   |
|                                  |       |     |                    |                  |                                  | 64.9                     | (1)                   |

Brittle fracture in, or near test piece head.

We claim:

1. A titanium-base alloy consisting of 2-10% by weight of chromium and 0.5-2% of boron, balance, apart from usual impurities, titanium. 35
2. A titanium-base alloy according to claim 1 consisting of 5% chromium and 1.2% boron, balance, apart from usual impurities, titanium. 40
3. A titanium-base alloy consisting of, by weight, 5% chromium and 0.8% boron, balance titanium with impurities. 45
4. A titanium-base alloy consisting of, by weight, 5% chromium and 1% boron, balance titanium with impurities. 50
5. A titanium-base alloy consisting of, by weight, 7% chromium and 1% boron, balance titanium with impurities. 50
6. A titanium-base alloy consisting of, by weight, 9% chromium and 1% boron, balance titanium with impurities.

## References Cited

## UNITED STATES PATENTS

- 2,596,489 5/1952 Jaffee et al. ----- 75—175.5  
2,726,954 12/1955 Jaffee et al. ----- 75—175.5  
2,754,204 7/1956 Jaffee et al. ----- 75—175.5  
3,199,980 8/1965 Brooks et al. ----- 75—175.5

## OTHER REFERENCES

Handbook on Titanium, WADC Tech. Rep. 54-305, August 1954, relied on pp. II-3-15 to II-3-19.

Titanium Project, "The Manufacture of Titanium Alloys," Navy Rep. No. 5, Oct. 20, 1950, Navy Contract No. NO a(s) 10683, relied on pp. 30-32.

Titanium Project, "The Manufacture of Titanium Alloys," Navy Rep. No. 9, Jan. 26, 1952, Navy Contract No. NO a(s) 51-006-C, relied on p. 45.

Titanium Project, "The Manufacture of Ductile Titanium and Titanium Alloys," Navy Rep. No. 17, Navy Contract No. NO a(s) 8698, relied on pp. 49-51.

DAVID L. RECK, Primary Examiner.

C. N. LOVELL, Assistant Examiner.